

# UNITED STATES PATENT OFFICE.

LEONARD F. DUNN, OF ONEIDA COMMUNITY, NEW YORK.

## PROCESS OF NICKEL-PLATING.

SPECIFICATION forming part of Letters Patent No. 289,337, dated November 27, 1883.

Application filed September 13, 1883. (No specimens.)

*To all whom it may concern:*

Be it known that I, LEONARD F. DUNN, of Oneida Community, in the county of Madison, in the State of New York, have invented new and useful Improvements in Process of Nickel-Plating, of which the following is a full, clear, and exact description.

In the art of nickel-plating articles of inferior metal it has been found that, although said plating presents a very hard surface and is capable of resisting, to a very great extent, abrasion and wear, and of receiving a high polish, yet the said metal is so brittle that when subjected to comparatively slight tensile strain it is caused to either peel off in large scales or fly in fine dust off from the article to which it has been applied as a plating. To overcome this defect I have prior to this resorted to the method of enveloping the nickel-plating between two coats of silver, as set forth in my Patent No. 278,784, dated June 5, 1883. Although this method accomplished to a great extent the desired object, it, however, proved somewhat expensive.

Having in my experiments discovered that by combining with the nickel-plating a plating of silver or copper or other ductile or malleable metal, the latter becomes more or less amalgamated with the nickel, and imparts thereto sufficient tensile strength to enable it to resist the strains incident to ordinary contortion of the article to which it is applied. I now apply the nickel-plating by interposing between two coats of said plating a plating of silver or copper or other ductile or malleable metal. The first coat of nickel may be either applied direct to the article to be plated or to a coat of other metal previously applied to said article. The plating of silver or copper or other ductile metal is next applied to the first coat of nickel, and then another coat of the latter is made to cover the plating of the ductile metal. This process of alternating the coats of nickel and of ductile metal can be continued to produce a plating of almost any desired thickness, said coating being applied by the ordinary electroplating process; and in practice I prefer to transfer the article under treatment from one bath to another as quickly as practicable, so as to expose the metal surfaces as little as possible to the atmosphere, and prevent the solution of one bath from becoming dry on the article before

the application thereto of the next solution. The ductile metal coating, which is thus interposed between the two nickel-platings, becomes to a great extent amalgamated therewith, and while forming a thorough tie of the several layers it at the same time imparts to the nickel-plating a degree of ductility which enables it to withstand considerable tensile strain.

I am aware that prior to my invention various methods have been resorted to to apply platings of precious metal to articles of inferior metal. In one instance a nickel coating has been applied directly to the inferior metal to form the base for a finishing coat of silver; in another case a silver coating has been first applied to the inferior metal, and after highly burnishing said silver coating a nickel-plating was applied thereto; and, again, in another case a film of tin has been combined with the nickel-plating electrically deposited; but it will be observed that neither of said prior methods produced a plating possessing the durability of the multiple coats of nickel united by, and to some extent amalgamated with, interposed thin coats of silver, as herein specified. Therefore

What I claim as new, and desire to secure by Letters Patent, is—

1. The method of nickel-plating inferior metal by interposing between two coats of nickel a coat of silver or other ductile metal, said coats being successively applied by ordinary electroplating process, substantially as set forth.

2. The process of nickel-plating inferior metal, consisting in applying by means of electrolysis alternate coats of nickel and coats of ductile metal, ending with a coat of nickel, and in applying the successive coats, transferring the article under treatment from one bath to the other without exposing the metal surfaces to the action of the atmosphere, substantially as set forth.

In testimony whereof I have hereunto signed my name and affixed my seal, in the presence of two attesting witnesses, at Syracuse, in the county of Onondaga, in the State of New York, this 3d day of September, 1883.

LEONARD F. DUNN. [L. S.]

Witnesses:

FREDERICK H. GIBBS,  
WM. C. RAYMOND.